

Jan. 17, 1950

R. F. ARNOLDY

2,494,791

OXIDATION OF THE HARDENED INNER SURFACE OF A PUMP  
LINER TO FACILITATE ITS REMOVAL FROM THE LINER

Filed Oct. 29, 1943

3 Sheets-Sheet 1



Fig. 1.

Inventor

R. F. ARNOLDY

By

Lester B. Clark.

Attorney

Jan. 17, 1950

R. F. ARNOLDY

2,494,791

OXIDATION OF THE HARDENED INNER SURFACE OF A PUMP  
LINER TO FACILITATE ITS REMOVAL FROM THE LINER

Filed Oct. 29, 1943

3 Sheets-Sheet 2



Inventor  
R. F. ARNOLDY

Lester B. Clark.

Attorney

Jan. 17, 1950

R. F. ARNOLDY

2,494,791

OXIDATION OF THE HARDENED INNER SURFACE OF A PUMP  
LINER TO FACILITATE ITS REMOVAL FROM THE LINER

Filed Oct. 29, 1943

3 Sheets-Sheet 3



Fig. 4.

Inventor

R. F. ARNOLDY

By

Lester B. Clarke

Attorney

## UNITED STATES PATENT OFFICE

2,494,791

## OXIDATION OF THE HARDENED INNER SURFACE OF A PUMP LINER TO FACILITATE ITS REMOVAL FROM THE LINER.

Roman F. Arnoldy, Houston, Tex.

Application October 29, 1943, Serial No. 508,266

1 Claim. (Cl. 148—13.1)

**1** In various arts tubular members are used wherein the internal periphery is coated with a hard surface material to resist wear of reciprocating parts or flowing fluids therein. Very often this hard surface becomes worn, irregular, or unserviceable for some reason or other and it is desirable to rework this surface so as to obtain additional use of the member itself. The invention has particular application to what are known as slush pump liners which is the inside liner of a reciprocating pump used for the circulation of an abrasive slush and mud in the rotary method of drilling wells.

The piston reciprocates in these liners, pumping a medium of abrasive material and the liner is subjected to considerable wear and often becomes scored or worn in such a manner that it is no longer serviceable. These liners come in various sizes and it has been found that if the hard internal surface can be economically removed, then the surface can then be reworked and provided with an additional hardened face of a slightly larger diameter than the original liner and that under these circumstances the liner can again be put in service.

The hard surfacing referred to may or may not be a ferrous metal in combination with chromium or boron and nickel. Other types include cobalt, chromium, tungsten alloys and boron bearing steels or other suitable materials. For purposes of illustration these will be generally designated as hardsurfacing or facing materials which will oxidize, but it is intended that this term shall apply to any of these hard surfacing materials. One rather general composition may be substantially 89% of iron, 4.8% of nickel, 3.2% of carbon and .8% of boron. Other types of hard wear resistant substances may be used so long as it is a material which may be treated with a temperature below the melting point of the base metal such as steel of the liner.

It is one of the objects of the invention to treat a tubular member having a hardened surface in such a manner that the surface is destroyed insofar as the composition of the hard material is concerned, with a view to reducing the hard material to a different composition which may be softer in the scale of hardness or which, because of its physical structure can be readily machined in order to remove the layer of such material from the inside of the liner or tubular member.

Another object of the invention is to oxidize a hardened surface inside of a tubular member so as to facilitate its removal.

**2** Another object of the invention is to treat a surface of hardened material by heating it to approximately 2000° F. and then forcing a stream carrying an excess of oxygen over the surface so as to effect the oxidation thereof and a change in the composition of the surface in order to facilitate its removal.

Other and further objects of the invention will be readily apparent when the following description is considered in connection with the accompanying drawings, wherein:

Fig. 1 is a central vertical sectional view of a furnace and illustrating the general arrangement and construction of the parts.

15 Figs. 2 and 3 are sections taken on the line 2—2 and 3—3 respectively of Fig. 1.

Fig. 4 is a sectional view similar to Fig. 1 but showing a modified arrangement for radiation or distribution of the heated fluids against 20 the liner surface.

While the invention will be described in detail and applied to a slush pump liner, it is to be understood that the process and apparatus may be applied equally as well to any type of 25 tubular member which is provided with a hardened surface, either on the inside or the outside thereof.

The furnace used in treating the liners is best seen in Fig. 1 and comprises a base 2 which may be made up in any suitable manner, that shown 30 being composed of channels 3 which have been filled with a concrete 4. It seems obvious, however, that any type of covering or supporting surface can be used upon these channels 3. This base is seen in Fig. 2 as being rectangular but it may be of any size or shape. Disposed upon this base is a floor 5 made up of two layers of 35 suitable fire-proof bricks or members 6.

These bricks are shown as arranged in opposite direction so as to form a sturdy support for the wall sections 7 and 8 which are disposed thereon.

The lower wall section is made up of a plurality of courses of fire-brick, which are shown 45 in Fig. 2 as being of a shape that they may be arranged in circular arches 10, four of which are seen in Fig. 2. It will be noted that these fire-brick are tapered with the narrow face inward so as that a plurality of them will form a suitable surface.

The inside arch or tier 11 of these bricks defines a mixing chamber 12 which is circular and of a length equal to the height of the two 50 courses of the bricks.

Fig. 2 shows this mixing chamber 12 as having the entries 13 and 14 thereinto from the flues 15 which extend to the outer periphery 17 of the wall section.

These flues 15 are arranged to form a passage for the products of combustion from the burners 18 which are shown as being directed into the passage by the lines 19. The burner 18 is seen in elevation in Fig. 1 and has a plurality of openings 20 therein so that a uniform blast of heated gases will be directed into the flue 15.

It should be noted that these flues 13 and 14 enter the mixing chamber 12 in a tangential direction so as to set up a circular or whirling motion of the gases in the chamber. These gases will rise and pass out of the top of the mixing chamber 12.

In order to provide a blast of air and an excess of oxygen in the mixing chamber to pass into the liner thereabove, an additional inlet 23 is provided in the form of a pipe of considerable diameter which passes through the base 2, the floor 5, and enters the chamber 12 in an axial direction. This blast of air may be suitably heated at a source not shown so that it may approximate a temperature of the gases entering the mixing chamber from the burners or the reaction and heat present in the chamber may effect the heating thereof.

It seems obvious that the air may be turned into the mixing chamber as desired, either before, during or after the heating by the fire from the burners.

The upper wall section 8 is very similar to the lower section 7 except that there are three arches of fire-brick and the heating or treating chamber 30 is somewhat larger in diameter than the mixing chamber 12 and is of a greater length. The length and diameter of this chamber will depend on the liner or other member which is to be treated.

The area between the chambers 12 and 30 is a stepped construction providing a shoulder 31, which forms a seat for the member which is to be treated.

Fig. 1 shows the liner 32 as having its lower end 33 seated on this shoulder 31 so that the gases and heated air from the mixing chamber 12 will be directed through the inside passage or area 33 in the liner.

In order to hold the liner 32 in proper position and to restrict the escape of the heated gases and air from the liner, a cap or cover plate 35 is shown as fitted into the upper end of the chamber 30. The handle 36 facilitates the insertion and removal of this cap or cover and the outlet passage 37 is shown as considerably restricted in order to confine the heat to the liner for the desired period.

It may be desirable to prevent any oxidation to the outer surface 40 of the liner while it is disposed in the chamber 30 and to this end an inlet 41 controlled by a valve 42 has been provided so that a suitable gaseous or liquid fluid may be applied to the outside of the liner and to fill the annular space 43 around the outside of the liner so as to prevent the oxidation thereof. Any suitable gas or liquid may be applied to this area to afford this protection.

The apparatus just described will be used and the method may be practiced by depositing the liner in position as shown in Fig. 1 and then turning on the burners so as to apply heat to the mixing chamber and to the inside of the liner.

As one illustration of the method, the temperature inside of the liner may be raised to 1900 or 2000° F. and after this temperature has been attained, hot air at approximately the same temperature will then be provided through the pipe 23 so as to introduce an excess of oxygen. This excess of oxygen is desired in order to oxidize the inner surface of the liner or other member and as an illustration of the time required with an ordinary size slush pump liner, the period of application of this hot air may be forty minutes to one hour. After this treatment the liner may be allowed to cool or may be removed so as to cool in air. No quenching of the liner is desired.

It has been found that this treatment of the liner or other member affects the hard surface. The excess of oxygen burns out the certain elements of the surface such as chromium, boron, carbon, etc. This leaves the surface or remaining material in a form which is much softer than or in a different physical state than the original hard surfacing material which was in place on the member at the time the treatment was started. This surface may be in the form of a scale which may be readily be removable.

This treatment results in the removal and/or destruction of the hard material and the next step after the cooling of the member is to then machine or otherwise remove the internal surface so as to remove such scale which results and to leave the surface in condition of a resurfacing operation or to machine it for use.

Another procedure may be to commingle the gas with an excess of air and introduce them simultaneously in order to provide an excess of oxygen to carry out the reaction. Thus sufficient oxygen is present for both combustion and reaction.

It might be well to state that it is the usual practice in manufacturing these liners to make the wall of a considerable thickness so that the liners may be used for the smaller size originally and then they may be enlarged by reborning or relining on several occasions so as to obtain the maximum of life and service from each individual liner. Of course when the liner is resized, then oversized pistons or other members which work in the liner will be used.

With liners which have been surfaced with these hard materials which are not readily machinable, it has been difficult to reuse the liners after the surface became worn or scored. The cost and trouble required to remove a hard surface such as has been applied to these liners was not only difficult, but uneconomical. By the treatment described herewith, it seems obvious that the hard surface is reduced to a softer surface which can be readily machined and the entire operation carried on satisfactorily so as to rework and reclaim the liner or other tubular member.

It is believed that the property or character of the hard material constituting the surface of the member is changed to another state. The thickness of this hard surfacing material may vary from .030 to .060 of an inch and the treating process is intended to be applied for a sufficient period of time to break up a surface of this thickness and to a depth such as will penetrate the hardened material to facilitate its removal.

Fig. 4 shows a slightly modified form of the furnace wherein the parts are the same as shown in Fig. 1 except for the cap member 35 which has been slightly modified so as to provide for a

somewhat larger opening as at 50 which more nearly approaches the inside area of the liner as at 33.

In some instances it may be that this area 33 is so large that the heated gases passing into the liner do not come in intimate contact with the surface 32. With a view of reducing the area for passage of the gases and also to force the gases into more intimate contact with the surface 32 a support plate 51 has been provided having the handles 52 thereon to permit the handling thereof, and arranged with a rod or projection 53 which is shown in Fig. 4 as extending the full length of the liner. This projection may be made of a refractory material and as will be seen in Fig. 4 it causes the heated gases flowing from the burner 13 to be forced radially outward against the inside surface of the liner so that the heat will be radiated back and forth between the projection and the surface of the liner as such gases move upwardly through the liner. It has been found that a conductor of this sort greatly facilitates the heating operation as to the amount of heat required and the time of heating. The other parts of Fig. 4 are the same as previously described.

It seems obvious that any hard facing material which is affected by a temperature below the melting point of the liner can be utilized and that heat as well as the oxidizing action may be used in combination together and the outside surface may be protected by a non-oxidizing atmosphere. The process has been particularly successful in the treatment of ferrous material containing boron.

Broadly the invention contemplates a method for treating slush pump liners and other tubular

members which have been hard surfaced and where it is desired to remove such surface and possibly replace it with a harder surface having a slightly different size.

What is claimed is:

In the process of removing the boron-carbide hard surfacing from the inner periphery of the boron bearing base metal of a pump liner the steps of, heating the liner to approximately 2000° F, and passing air, heated to approximately the same temperature, through the inside of the liner for approximately forty minutes, whereby the carbide is converted to an oxide which can thereafter be readily removed.

ROMAN F. ARNOLDY.

#### REFERENCES CITED

The following references are of record in the file of this patent:

#### UNITED STATES PATENTS

| Number    | Name         | Date           |
|-----------|--------------|----------------|
| 745,432   | Gohn         | Dec. 1, 1903   |
| 899,285   | Bert         | Sept. 22, 1908 |
| 1,404,001 | Barrett      | Jan. 17, 1922  |
| 1,416,865 | Patch        | May 23, 1922   |
| 1,898,809 | Berg         | Feb. 21, 1933  |
| 1,901,804 | Davis et al. | Mar. 14, 1933  |
| 2,034,822 | Morrow       | Mar. 22, 1936  |
| 2,081,612 | Woodson      | May 25, 1937   |
| 2,097,298 | Meyers, Jr.  | Oct. 26, 1937  |
| 2,116,228 | Akin         | May 3, 1938    |
| 2,125,172 | Kinzel       | July 26, 1938  |
| 2,356,329 | Lundbye      | Aug. 22, 1944  |

#### OTHER REFERENCES

Automotive Industries Magazine, Dec. 1, 1939, page 592.